

June 24, 1958

H. J. OKOOMIAN ET AL

2,840,500

HEAT INSULATING SHEET OR PANEL

Filed Dec. 22, 1954

2 Sheets-Sheet 1

FIG. 1.



FIG. 2.



FIG. 3.



FIG. 4.



FIG. 6.

INVENTORS

Howard J. Okoomian  
Lovic P. Herrington

BY Campbell, Brumbaugh, Tree & Grimes

THEIR ATTORNEYS

June 24, 1958

H. J. OKOOMIAN ET AL

2,840,500

HEAT INSULATING SHEET OR PANEL

Filed Dec. 22, 1954

2 Sheets-Sheet 2

FIG. 5.



FIG. 7.



FIG. 8

INVENTORS

Howard J. Okoomian  
Lovic P. Herrington.

BY Campbell, Brumbaugh, Tree & Graves

THEIR ATTORNEYS

# United States Patent Office

2,840,500

Patented June 24, 1958

1

2,840,500

## HEAT INSULATING SHEET OR PANEL

Howard J. Okoomian, West Haven, and Lovic Pierce Herrington, Hamden, Conn., assignors to John B. Pierce Foundation, New York, N. Y., a corporation of New York

Application December 22, 1954, Serial No. 476,892

8 Claims. (Cl. 154—44)

This invention relates to insulating sheets or panels, and in general aims to provide a panel which is a highly efficient heat insulator. Ancillary objects are to provide a heat insulating panel which is flexible so that it may be bent to conform to curved surfaces, yet sufficiently resilient that it will spring back to its original shape when the bending stress is relieved, which is made of readily available or non-strategic materials, which may be easily secured to walls, ceilings and other supports by ordinary fastening elements such as nails, staples or bolts, which is light in weight, is not too bulky being in fact nestable, is sufficiently stiff to be easily handled, will withstand extremes of climate, is fire-resistant, will not rot or corrode in moist air or be attacked by fungi, and if necessary may be washed. All these qualities make the panel of our invention a desirable wall surface for the interiors of temporary or portable buildings such as the Army must use in many parts of the world for personnel and supplies. Other advantages of our panel arise from the fact that aluminum foil is preferably used as facing sheets for the panel in order to reflect radiant heat; this foil reflects a good deal of light also, which results in a much brighter interior for the building wherein the panels are placed as components of an interior wall. A better illuminated interior is desirable to enhance morale and to diminish the use of artificial lights during daylight hours. Also the foil preferably has a surface such that it presents a pleasing, even a handsome appearance. The invention is also characterized by other objects and advantages.

With reference to the invention, in the case of a laminate insulating panel composed of an inner layer of insulating material (such as glass wool) and one or more outer layers of heat-reflecting sheets (such as metal foil), it has always been assumed by the prior art that the inward facing surfaces of the sheets, when in contact with filler insulation, have no important reflective insulation effect, since any such effect is assumed as necessarily dissipated due to the direct heat conduction path between the inner metal surfaces afforded by filler insulation, or due to the prevention of reflection when paper or other material is in direct contact with the metal surface. This being the assumption, it was customary in the prior art, for constructional reasons, to thermally short circuit or to reduce or eliminate the heat reflectivity of these inner sheet surfaces by coating them overall with adhesive to bond the sheets to the central layer, by placing a paper layer in direct contact with the inner sheet surfaces between the sheets and the central layer, or by like practices.

We have found, contrary to this prior art assumption, that the inward facing surfaces of the heat-reflecting sheets do, in fact, add considerably to the insulating capabilities of the panel, providing that the proper precautions are taken against thermal short circuiting of these inner surfaces by heat conduction.

The case in which no thermal short circuiting (by heat conduction) whatever would occur is that arrangement in which the inner surfaces of the sheets are separated only by an air gap. Such arrangement is not desirable, however, for the reason that convection currents in the air gap would reduce insulating efficiency, and for the further reason that the arrangement is not practical constructionwise.

2

In order to meet these difficulties it is necessary, in constructing a panel to use an insulating material as a filler between the heat-reflecting sheets. At the same time, in order to take advantage of the insulating powers of the inner sheet surfaces, it is important to keep the thermal short circuiting of these surfaces to a minimum by reducing, insofar as possible, the areas where the surfaces are directly contacted.

The amount of such direct contact is minimized in accordance with the present invention by (1) avoiding the use of paper layers or the like between the metal sheets and the central insulating layer, (2) restricting to limited areas the adhesive which bonds the sheets and central layers together, (3) using a fibrous central insulating layer with a medium density offering a balance between a low total contact area of the fibers with the sheets and a satisfactory constructional strength, and (4) forming a multiplicity of ridges and valleys in the panel to further reduce the contacts between the central layer fibers and the sheet inner surfaces.

It is thus seen that a panel in accordance with the invention represents an optimum balance between the features increasing the insulating powers of the panel and the features desirable from a construction point of view. 10 15 20 25 30 35

In this connection it will be understood that the word "panel" as used herein refers generally to an insulating structure of relatively large extent in two dimensions thereof compared to the third dimension thereof. Thus, the description of the present invention as a "panel" is not to be construed as limiting the invention to structures suitable only to perform a wall paneling function.

The invention will be better understood from the following description of the preferred embodiment of the invention shown in the accompanying drawings forming 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885

terial since it is a good infra-red as well as visible light reflector, resists atmospheric corrosion, is sufficiently stiff to partially maintain its own shape and is to some extent resilient in flexure, adding thereby to the resiliency of the whole panel. The last two-named properties of aluminum foil permits a lower density glass wool layer to be used to attain the advantages heretofore mentioned.

In lieu of aluminum foil, more expensive foils or sheets having like properties, e. g. chromium, could be used.

The fibrous core 10, in the finished and preferred form of panel, is about 0.31 to 0.33 in. thick while the facing foil sheets 11, 12 are about 0.006 in. thick but may be as thin as 0.003 in. The entire laminate is corrugated, with the corrugations parallel and of the same dimensions, preferably of about  $\frac{5}{8}$  in. to  $\frac{3}{4}$  in width. By making the width of the core of about the same size or less than the length of the sides of the corrugations, the susceptibility to flexure of the presently disclosed panel is increased to panels where the opposite situation obtains.

The corrugations of the foil sheets 11, 12 preferably have their walls at angles of  $90^\circ$  (Fig. 3) or  $60^\circ$  (Fig. 6) to each other. These corrugations are of serrate form in that they present a multiplicity of sharp-angled peaks or ridges 13 alternating with valleys or depressions 14, the respective corrugations of the two sheets registering angle for angle with each other so that the centers of the valleys of one foil sheet extend toward (that is, are in the same planes as) the peaks of the foil sheet on the other side of the core 10. Thus core 10 itself is of corrugated serrate form and a substantially uniform thickness at all points. Preferably the aluminum foil of sheets 11 and 12 is crimped to present flattened waves 15 which extend at right angles to the direction in which peaks 13 extend. These waves reflect light in two directions to improve the distribution of light reflected from the panel when the same is used to brighten a building interior. Also the waves give a striped appearance to the panel which materially enhances the appearances of the panel. The waves 15 may, however, extend parallel to the peaks 13.

It will be seen that forming the panel to have a multiplicity of folds, either as corrugations or as waves 15, reduces the amount of direct contact between the inner sheet surfaces and the glass wool fibers, since the fibers in their distribution tend to be less concentrated at the angles of the folds. In this regard the size of the corrugations and crimping waves of the presently described panel are believed to represent the optimum balance between the case where the folds are so numerous as to approach a flat surface and the case where the sheet inner surfaces are, in fact, flat surfaces. Moreover, either one or both of the corrugation or crimping folds serve (as an effect independent of reduction of direct contact with the filler material) to enlarge greatly the area of inner reflective surface over that afforded by a flat sheet. Thus the folds considerably increase the radiant insulation power of the sheets. Exterioly, such folds minimize the physical contact of the outer reflecting surfaces with any other surfaces supporting the panel when applied to, say, a building or a pipe. The reduction in exterior physical contact serves, like the mentioned reduction in interior contact, to minimize the loss of insulating power by direct solid conduction of heat and to maximize the radiant insulating effect of the outer surfaces.

A panel made as described may have a density of about 6.1 lbs. per cubic foot, an over-all thickness of about 1.05 in., and at  $139^\circ$  F., a conductance of 0.487 B. t. u./hr./ $^\circ$  F./sq. ft. and a thermal resistance of 2.05 B. t. u./hr./ $^\circ$  F./sq. ft. The "Clo" per inch of glass wool (.31 in. thickness) equals 7.54 and the resistance per inch of glass wool equals 6.61 B. t. u./hr./ $^\circ$  F./sq. ft. 75

To hold the glass wool core against shifting during handling of the panel, and to make an easily handled assembly or laminate, the glass wool is coated along narrow areas with polyvinyl chloride adhesive, or other adhesive, as indicated at 16, 17, 18, 19 and 20 in Fig. 1, thereby uniting the metal foil sheets to the core. These narrow areas of adhesive are preferably only about one inch wide and extend preferably along the edges of the panel and in straight lines parallel to one of the long panel edges, as shown in Fig. 1. If the panel is narrow, the intermediate adhesive area 20 may be omitted.

As stated, by bonding the glass wool layer and foil sheets together by only a few narrow bands of adhesive, the heat transference through the panel is minimized compared with the case where the adhesive is distributed over the major portion of the reflective surface in a uniform layer. As another advantage over uniform layer distribution, an adhesive substance used to bond panels of the sort described, generally stiffens the panels where applied. Hence, by applying the adhesive in only a few narrow bands the panel is rendered more readily susceptible to resilient flexing.

The dimensions shown in Fig. 1 are merely illustrative; obviously the panel may have any length and width that permits convenient handling by one or two operators. The described panels may be bent as much as  $90^\circ$  about an axis A as Fig. 5 shows, to accommodate the panel to curved walls. After the bending stress has been removed, the described panel will resume its original form because of its resiliency.

Among the factors contributing to the over-all flexural susceptibility and resiliency of the panel are the following: (1) the resiliency of the core itself, (2) the resiliency of the foils, (3) the relative width of the core compared to the length of the sides of the corrugations, (4) the restriction of the adhesive to only a few narrow bands.

There are at least two methods which may be followed in fabricating the described panels. The metal foil sheets may be passed over adhesive rolls or applicators to apply the adhesive in narrow strips or areas as described and then brought into contact with a glass fiber batt, following which the assembly may be crimped to assume the corrugated form shown in Fig. 3 or Fig. 6. Such crimping will be done by power-driven rolls, as will be understood by those skilled in the art. Another method involves corrugating the glass wool core first, and then applying the metal foil with pressure to make the sheets conform to the corrugated core. This method is especially useful with very thin foils (about .003 in.), the necessary dimensional stability of the panel being achieved through a glass wool core that has been stiffened by means of a resin. Obviously by varying the fiber diameter and the amount of binding resin, almost any degree of rigidity in the panel may be obtained. Very thin foils not only reduce the weight of the panel but also have the same insulation efficiency as heavy foils or thin sheets which are much more expensive. Of course, very thin foils are easily damaged in handling.

The following table is based on comparative tests of the described panel (sample No. 9) with other sheets and laminates (described below).

Table

| Sample No. | Conductance | Resistance | Thickness of Glass Wool (in.) | Resistance per inch of Glass Wool |
|------------|-------------|------------|-------------------------------|-----------------------------------|
| 1          | .232        | 4.31       | 1.24                          | 3.48                              |
| 2          | .404        | 2.48       | .62                           | 4.00                              |
| 3          | .447        | 2.24       | .62                           | 3.61                              |
| 4          | .275        | 3.64       | .98                           | 3.71                              |
| 5          | .424        | 2.36       | .62                           | 3.81                              |
| 6          | .479        | 2.09       | .62                           | 3.37                              |
| 7          | .435        | 2.30       | None                          | -----                             |
| 8          | .743        | 1.35       | None                          | -----                             |
| 9          | .487        | 2.05       | .31                           | 6.61                              |
| 10         | .620        | 1.61       | .31                           | 5.19                              |

NOTE.—Limiting resistance for 1 in. of absolutely still air is 5.2 (Smithsonian Physical Tables, F. E. Fowle, Smithsonian Institution, 1934).

Sample No. 1 of the above table consisted of two layers of glass wool between which was a sheet of corrugated aluminum foil .006 in. thick attached at the tops of the corrugations to the glass wool by polyvinyl adhesive. Sample No. 2 consisted of two sheets of corrugated aluminum foil .006 in. thick between which was a layer of glass wool adhered by adhesive to the tops of the corrugations. Sample No. 3 consisted of a sheet of corrugated aluminum foil .006 in. thick adhered by adhesive applied at the tops of the corrugations to a layer of glass wool. Sample No. 4 was commercial glass wool, and sample No. 5 was the same but of less thickness. Sample No. 6 was like No. 5 except that the glass wool layer on both sides had a facing of  $1/16$  in. crimped aluminum foil adhered thereto. Sample No. 7 was merely a single sheet of corrugated aluminum foil such as was used in the laminates identified as samples 9 and 10. Sample No. 8 was like No. 7 but with different air spacing. Sample No. 9 embodied the invention herein described. Sample No. 10 was like No. 9 except the two reflective surfaces on the inside of the two aluminum foil sheets were blackened with black paint to eliminate reflectance from these surfaces. This sample also embodied the invention, even though the elimination of reflectance was a step backward.

It will be observed that sample No. 9 materially exceeded the limiting value of absolutely still air, and even sample No. 10 almost equalled such value (5.19 nearly = 5.2).

In order to make the described panel conform to a curvature or bend in a wall or ceiling it may be turned so that the corrugations extend either horizontally or vertically. When the corrugations run horizontally, the panel may be bent in a vertical plane, while if the corrugations extend vertically, the panel may be curved in a horizontal plane. Tacks, nails, staples, etc. are easily driven through the panel, and because of its dimensional stability, comparatively few fastening elements are needed to hold it in position, which is advantageous especially in very cold weather, when frost will build up on metallic fastening elements. When the panel is secured against a flat surface, it will touch that surface only along the sharp peaks or ridges of the corrugations, which is advantageous in greatly reducing conduction.

When shipping the panels, much space may be saved by nesting them, as will be apparent from Fig. 7. Such nested panels of two, three, or more layers, coupled together by mechanical fastening elements such as staples or by adhesive along the edges, will form insulating layers useful in various structures, e. g., refrigerators, refrigerator cars or trucks, temporary or permanent buildings, etc. This nesting feature may also be useful in closing the joints made by two abutted panels, since narrow strips ( $3\frac{1}{2}$  in. or  $4\frac{1}{2}$  in. wide) cut from the panels may be placed over such joints to conceal and substantially to seal them, especially if polyvinyl adhesive or the like is used to hold the strips tightly against the joints with the corrugations of the strips nested into the corrugations of the abutted panels. This will be understood without specific illustration.

An even more efficient insulating wall structure is shown in Fig. 8, where two panels 30, 31, exactly like the panel of Figs. 15, are spaced apart by means of a woven or meshed fabric 32 which may be of galvanized wire, asbestos netting, or even plastic or glass fiber cloth. Adhesive or fastening elements may secure the fabric to the panels. As fabric 32 prevents contact between the reflective surfaces of the foil, and as the peaks and valleys are directly opposed, a multiplicity of reflective dead air spaces 33 are provided which would operate as a resistance in series with the panels. Fabric 32 is of course very flexible to permit bending. The principal

disadvantage of the arrangement of Fig. 8 is its much greater over-all thickness as compared to the nested arrangement of Fig. 7. As more of the panels can be assembled in the same wall space, if they are nested as in Fig. 7, the latter arrangement may be preferred in some cases even though less efficient in resistance for an equal weight of material.

From the foregoing, it is clear that our invention provides a panel or insulating construction which is a better heat insulator than absolutely still air. The reason for the excellence of our heat-insulating panel lies in maximizing the use of the reflective principle of insulation with a fibrous filler material which reduces internal convection to a minimum without destroying the reflective insulation effect of the internal foil surfaces.

The above-described embodiments being illustrative only, it will be understood that the invention comprehends organizations differing in form or detail from the described embodiments. Also constructions according to the invention

may be used not only as wall panels, but in divers other ways. For example, a two inch diameter pipe heated to 300-700° F. would normally take an additional inch of insulation on each side, increasing the over-all covered diameter to four inches. With an insulating jacket of a construction according to the invention, the jacket on each side would take up only 0.6 inch of diameter to reduce the over-all covered diameter of the insulated pipe to 3.2 inches.

Accordingly, the invention is not to be considered as limited save as is consonant with the scope of the following claims.

We claim:

1. A heat insulating panel comprising, a pair of bright metallic foil, heat reflecting sheets each having inner and outer heat-reflecting surfaces and each having a plurality of similar sharp angle corrugations which extend in the direction of their ridge lines normal to a plane passing through both sheets and which follow on each other in juxtaposed relation in said plane to render the cross-sections of said sheets in said plane of the same sawtooth shape, said sheets being mutually separated with respective corrugations thereof registering angle for angle and with corresponding faces of registering corrugations being parallel to thereby define between said sheets an interspace having in said plane a cross-section of sawtooth shape and of an inter-sheet width less than the dimension in said plane of the face of one of said corrugations, and a layer of fibrous glass wool occupying substantially all of said sawtooth-shaped interspace to the exclusion of air pockets therein, said glass wool layer and said sheets being bonded together to form a united panel structure.

2. The invention defined in claim 1 wherein the interior angles of the corrugations are about 90°.

3. The invention defined in claim 1 wherein the interior angles of the corrugations are about 60°.

4. A panel as in claim 1 wherein the two sheets are of aluminum foil .006 inch to .003 inch thick, the faces of the corrugations being from  $\frac{5}{8}$  to  $\frac{3}{4}$  inch long in the said plane, and wherein the central insulating layer is of glass wool of a thickness of about 0.3 inch.

5. A heat insulating panel comprising, a pair of bright metallic foil, heat reflecting sheets each having inner and outer heat-reflecting surfaces and each having a plurality of similar sharp angle corrugations of major size which extend in the direction of their ridge lines normal to a plane passing through both sheets and which follow on each other in juxtaposed relation in said plane to render the cross-sections of said sheets in said plane of the same sawtooth shape, said two sheets each having minor size ridges and valleys which run transversely to the major size corrugations of the sheets and said sheets being mutually separated with respective corrugations thereof registering angle for angle and with corresponding faces of registering corrugations being parallel to thereby define

between said sheets an interspace having in said plane a cross-section of sawtooth shape and of an inter-sheet width less than the dimension in said plane of the face of one of said corrugations, and a layer of fibrous glass wool occupying substantially all of said sawtooth-shaped interspace to the exclusion of air pockets therein, said glass wool layer and said sheets being bonded together to form a united panel structure.

6. A heat insulating panel comprising, a pair of bright metallic foil, heat reflecting sheets each having inner and outer heat-reflecting surfaces and each having a plurality of similar sharp angle corrugations which extend in the direction of their ridge lines normal to a plane passing through both sheets and which follow on each other in juxtaposed relation in said plane to render the cross-sections of said sheets in said plane of the same sawtooth shape, said sheets being mutually separated with respective corrugations thereof registering angle for angle and with corresponding faces of registering corrugations being parallel to thereby define between said sheets an interspace having in said plane a cross-section of sawtooth shape and of an inter-sheet width less than the dimension in said plane of the face of one of said corrugations, a layer of fibrous glass wool occupying substantially all of said sawtooth-shaped interspace to the exclusion of air pockets therein, and adhesive material disposed between said glass wool layer and each of said sheets and distributed over the area of said panel to extend parallel to the ridge lines of said corrugations only in narrow bands adjacent the edges of said panel, and to extend transverse to said ridge lines only in narrow bands, said adhesive material bonding said sheets and layer together into a united panel structure.

7. A heat insulating panel comprising, a pair of bright metallic foil, heat-reflecting sheets each having inner and outer heat-reflecting surfaces and each having a plurality of similar sharp angle corrugations of major size which extend in the direction of their ridge lines normal to a plane passing through both sheets and which follow on each other in juxtaposed relation in said plane to render the cross-sections of said sheets in said plane of the same sawtooth shape, said two sheets each having minor size ridges and valleys which run transversely to the major size corrugations of the sheets and said sheets being mutually separated with respective corrugations thereof registering angle for angle and with corresponding faces of registering corrugations being parallel to thereby define between said sheets an interspace having in said plane a cross-section of sawtooth shape and of an intersheet width less than the dimension in said plane of the face of one of said corrugations, a layer of fibrous

glass wool occupying substantially all of said sawtooth-shaped interspace to the exclusion of air pockets therein, and adhesive material disposed between said glass wool layer and each of said sheets and distributed over the area of said panel to extend parallel to the ridge lines of said corrugations only in narrow bands adjacent the edges of said panel, and to extend transverse to said ridge lines only in narrow bands, said adhesive material bonding said sheets and layer together into a united panel structure.

8. A heat insulating assembly comprising a first heat insulating panel including a pair of bright metallic foil, heat reflecting sheets each having inner and outer heat-reflecting surfaces and each having a plurality of similar sharp angle corrugations which extend in the direction of their ridge lines normal to a plane passing through both sheets and which follow on each other in juxtaposed relation in said plane to render the cross-sections of said sheets in said plane of the same sawtooth shape, said sheets being mutually separated with respective corrugations thereof registering angle for angle and with corresponding faces of registering corrugations being parallel to thereby define between said sheets an interspace having in said plane a cross-section of sawtooth shape and of an inter-sheet width less than the dimension in said plane of the face of one of said corrugations, and a layer of fibrous glass wool occupying substantially all of said sawtooth-shaped interspace to the exclusion of air pockets therein, said glass wool layer and said sheets being bonded together to form a united panel structure; said assembly further comprising a second heat insulating panel similar to said first panel and a flexible fabric interposed between said panels with opposite surfaces of said fabric making contact with ridge lines of the respective corrugations of said panels, said corrugation ridge lines of said two panels being in opposed relation through said fabric so that air spaces are provided between said panels.

#### References Cited in the file of this patent

#### UNITED STATES PATENTS

|           |               |               |
|-----------|---------------|---------------|
| 1,186,572 | Guibert       | June 13, 1916 |
| 2,057,071 | Stranahan     | Oct. 13, 1936 |
| 2,083,596 | Donley        | June 15, 1937 |
| 2,230,823 | Batcheller    | Feb. 4, 1941  |
| 2,540,331 | Hlavaty       | Feb. 6, 1951  |
| 2,576,698 | Russum        | Nov. 27, 1951 |
| 2,644,777 | Havens        | July 7, 1953  |
| 2,671,492 | Biordi et al. | Mar. 9, 1954  |
| 2,746,892 | Elfving       | May 22, 1956  |